

W. R. SEIGLE,  
METHOD OF FORMING TUBES OF FELTED FIBROUS MATERIAL,  
APPLICATION FILED JUNE 28, 1920.

1,399,087.

Patented Dec. 6, 1921.



Fig. 2.



1399087  
William R. Seigle  
By John Louis Schumacher  
ACROSS SEIGLE

# UNITED STATES PATENT OFFICE.

WILLIAM R. SEIGLE, OF NEW YORK, N. Y.

## METHOD OF FORMING TUBES OF FELTED FIBROUS MATERIAL.

1,399,087.

Specification of Letters Patent.

Patented Dec. 6, 1921.

Application filed June 28, 1920. Serial No. 392,372.

*To all whom it may concern:*

Be it known that I, WILLIAM R. SEIGLE, a citizen of the United States of America, and resident of New York, in the county of New York and State of New York, have invented new and useful Improvements in Methods of Forming Tubes of Felted Fibrous Material, of which the following is a specification.

0 My invention relates to the manufacture of wound paper or pulp tubes and has for its particular objects the construction of dense, thick walled tubes of larger diameter than have heretofore been obtainable, and 15 further, the construction of tubes of the aforesaid character from asbestos fiber or pulp.

This invention consists of a method of manipulating a web of fibrous material, 20 felted with water, by which the water contained in the web and associated with the fibers is so controlled and actuated as to be instrumental in incorporating successively superposed layers of the web with each other 25 into a substantially homogeneous single felted body, which exhibits none of the heterogeneity of discernibly laminated built-up fibrous sheets, and in the product of said method.

30 This method requires apparatus wherewith to carry it out; such apparatus is exemplified in a machine, herein described, which is also of my invention and by means of which I have been enabled to construct asbestos and 35 other fiber tubes of high and uniform density, because of those characteristics adapted when cut into suitable segments to serve as linings for brake-bands, especially when prepared for service by impregnation with 40 a cementitious, fiber reinforcing filler, such as a hardened oil. Such special products of the method and machine herein to be described form the subject matter of other applications for patent filed by me concurrently herewith, and serially numbered 392-, 45 373, and 392,374. The machine herein described also forms the subject matter of an application for patent, filed by me concurrently herewith, Serial No. 392,371.

50 In my United States Letters Patent numbered 1,037,670, dated September 3, 1912, there is described a pulp tube machine adapted to the construction of pulp tubes of high density and inherent strength, and the subject matter of the present specification descriptively includes functionally related fac-

tors substantially the same as those which characterized the invention set forth in the said patent.

Since one ultimate object of this present invention is the production of a material eminently suitable to serve as brake-band linings, homogeneity of the fibrous felted structure of the pulp tube or cylinder is a prime requisite. The desired homogeneity 65 is negatively characterized by practically complete absence of any stratifications or laminations in the wall of the pulp tube, and adapts the tubular structure to the reception and inclusion in its body, of impregnants 70 which, by their binding and cementitious effect on the fibers which are comprised in the tube-structure, transform it into a friction sustaining material of solid consistency throughout. In the drawings hereto annexed, which illustrate a machine by which one may perform the process of my invention—

Figure 1 is a diagrammatic elevation-view of a pulp-tube machine; and

Fig. 2 is a broken longitudinal section of the suction roll on which the pulp tube is wound.

The mechanical details of machines of the general character indicated are too well 85 known to require full illustration or explanation.

In Fig. 1, A indicates the pulp-tank, B the cylinder mold, C the felt, which is preferably thin, as and for the reasons described in my aforesaid Patent No. 1,037,670; D a thickly felted couch roll, which may be mounted on a pivoted frame, as D'; E a segmental roll, with the well-known suction commutator (not indicated) by means of 90 which suction is maintained between selected segment-partitions such as F, and relaxed between others; G represents the area over which suction is thus maintained; this area terminates near to, but short of the line of 100 tangency between the felt C and the mandrel roll, presently to be described; H, J, K, L and M are guide rolls for the felt C; and I, I are whip-rolls.

N represents the mandrel roll, on which 105 the pulp tube is wound. This is a continuous suction roll, and is connected to the branch P of the suction pipe O; this branch P may be corrugated as at O', or otherwise provided with means to permit the mandrel 110 roll N to bear heavily on the felt C, and to rise as the tube material accretes upon the

mandrel roll. The branch Q from the suction pipe O communicates with the interior of the segmental suction roll E. A compacting roll R, mounted on a pivoted frame 5 S, bears on the top of the mandrel roll N, or upon the pulp tube in the course of its construction. An adjustable weight T may be provided, wherewith to adjust the pressure with which the roll R bears upon roll 10 N, and consequently causes roll N to bear upon the felt C, supported by the segmental roll E.

The construction of the mandrel roll N is more fully illustrated in Fig. 2. It comprises an inner cylinder N', perforated at N<sup>2</sup>, and an outer jacket N<sup>2</sup>, of finely and closely perforated metal, or of wire cloth. The inner cylinder N' forms a substantially air-tight joint at N<sup>4</sup> with the head plates P' 15 (of which one is shown) so that it may rotate in relation to the head plates while suction is maintained within it. The outer jacket N<sup>2</sup> is provided with end sleeves, as N<sup>6</sup>, which make a substantially air-tight fit, as 20 at N<sup>5</sup>, with the imperforate portions of the inner cylinder N'.

The outer jacket N<sup>2</sup> provides the perforated or reticulated surface on which the pulp tube is wound. This jacket is removable from the inner cylinder N', so that when a pulp tube has been built up on the jacket, the jacket with the tube on it may be removed, and replaced by a similar jacket on which another tube is built.

35 The operation of the machine comprising the foregoing factors is as follows:

By means of the heavily felted couch roll D, a film or web of interlaced or felted fibers is taken off the cylinder mold B on to the 40 felt C and carried thereon to the segmental suction roll E. The suction maintained on this roll through the region indicated at G extracts a considerable portion of the water contained in the fibrous web, but is relaxed 45 at a point, or rather a line along the cylindrical surface of the roll which is far enough from the line of tangency of the mandrel roll M to permit the water remaining in the fibrous web to regain its outer surface and 50 moisten it, so that it unites intimately with layers previously wound upon the mandrel roll. This intimacy of incorporation of successive layers of fibrous web with each other is further insured by the continuous suction 55 maintained in the mandrel roll, which draws the fresh, wet and relatively mobile fibers into firm union with previously deposited fibrous layers, and at the same time by drawing water, carried to the outer layer by the 60 fibrous web coming from the felt C, through the whole accumulated mass of fiber, felting the fibers of successively applied layers together, so that upon completion, the pulp tube on the mandrel roll is in 65 every practical and substantial respect a

single homogeneous felted structure, free from the heterogeneity or lack of unity which characterizes structures formed of discernible or separable laminæ.

The compacting roll R contributes to the 70 density and homogeneity of the built-up pulp-tube by exerting pressure on the tube as it accumulates on the mandrel roll, both at the line of tangency of the roll R itself, and that of the mandrel roll N upon the 75 felt C.

When the pulp tube has acquired the desired thickness of wall, the machine is stopped, the jacket N<sup>2</sup> with the pulp tube unit removed from the perforated cylinder 80 N', and a similar jacket put on the cylinder, which is then remounted in the head plates P'. The formation of another pulp-tube is then begun.

After the pulp tubes have been cured by 85 drying to any desired extent, they can be slit longitudinally and removed from the jacket N<sup>2</sup>. It is not intended that these pulp tubes shall be taken from the jackets while moist and plastic, and be flattened 90 as is the practice in making mill-board and the like. The machine herein described is designed to produce pulp tubes of such thickness in relation to diameter that such flattening would be quite impracticable. As 95 to the product itself, a principal object of this invention is to construct dense, thick-walled pulp tubes which shall be allowed to dry and become set in cylindrical form, so that segments cut from such tubes shall be 100 of suitable shape and proportions to be attached to brake shoes and the like, and serve thereon as linings.

In general, pulp tubes comparable in respect to density and thickness of wall to 105 those manufactured on machines of the character described in my said Patent No. 1,037,670, but of much larger diameter than has been found practicable to attempt on such machines, can be produced by means of 110 the invention herein described.

The product of the above described method may be characterized as one of layer-accumulation, as distinguished from bodies made by compressing a mass of 115 fibrous material, with or without a filler or cementitious ingredient, *en bloc*, in a mold. Curved segmental bodies comprising fibrous material have been made, and used for brake shoes and the like, by the block-molding method, but that method is not adapted to the construction of segments which subtend large arcs; whereas the layer accumulation or layer-accretion method is adapted to the construction of segments which subtend arcs up to the complete circumference 120 of a circle.

I claim:

1. The method of forming tubes of fibrous material, which consists in forming 130

a web of said fibrous material with water, extracting part of the water-content from said web, superposing successive layers of said web on each other, and forcing part of the water remaining in said layers from the latest superposed layer thereof to and through the other layers.

2. The method of forming tubes of felted fibrous material, which consists in forming 10 a web of said fibrous material with water, extracting part of the water-content from said web, superposing successive layers of said web on each other under pressure, and forcing part of the water remaining in said 15 layers from the latest superposed layer thereof to and through the other layers.

3. The method of forming tubes of felted fibrous material, which consists in forming a web of said fibrous material with water,

extracting part of the water-content from 20 said web, superposing successive layers of said web on each other, and forcing by suction part of the water remaining in said layers from the latest superposed layer thereof to and through the other layers. 25

4. The method of forming tubes of felted fibrous material, which consists in forming a web of said fibrous material with water, extracting part of the water-content from 30 said web, superposing successive layers of said web on each other under pressure and forcing by suction part of the water remaining in said layers from the latest superposed layer thereof to and through the other layers. 35

Signed by me at New York, N. Y., this 25th day of June, 1920.

WILLIAM R. SEIGLE.